

Nov. 19, 1946.

J. R. McMILLIN ET AL

2,411,326

MAKING REINFORCED SLIVERS

Filed Nov. 27, 1942



## UNITED STATES PATENT OFFICE

2,411,326

## MAKING REINFORCED SLIVERS

James R. McMillin and Stanley H. Lake, Newark, Ohio, assignors to Owens-Corning Fiberglas Corporation, Toledo, Ohio, a corporation of Delaware

Application November 27, 1942, Serial No. 467,278

7 Claims. (Cl. 19—145)

1

This invention relates to a fibrous product and to an improved method and apparatus for manufacturing such a product.

In the manufacture of certain types of fibrous products such, for example, as glass or other thermoplastic materials, it has been customary to collect attenuated glass fibers on the periphery of a drum and to pull the deposited fibers off the drum to form a sliver of glass fibers. This method is disclosed and claimed in the Tucker and Lannan Patent No. 2,264,345, dated December 2, 1941.

Although slivers of the character disclosed in the above patent have proved very satisfactory in practice, nevertheless, in the manufacture of certain products, it is desirable to increase the tensile strength of the sliver. With this in view the present invention contemplates reinforcing the sliver with a continuous strand which may be a single filament or may be a yarn of desired material, preferably glass.

Heretofore reinforced asbestos slivers have been produced by feeding a reinforcing thread and an asbestos sliver together between the usual rubbing aprons or belts for condensing the sliver, and folding the sliver around the thread by the action of the belts. This process is not satisfactory in the treatment of glass fibers, however, because the use of rubbing aprons would represent an added, otherwise unnecessary step in the production of the slivers.

It is an object of the present invention to produce a reinforced glass sliver without increasing the number of steps or operations over those needed to produce an ordinary glass sliver.

More particularly this invention contemplates distributing glass fibers in tangled relation about a continuous strand of material as the fibers are produced, the strand being advanced along a predetermined path of travel coinciding with the movement of the sliver as it is formed, and, if desired, applying an adhesive to the strand prior to distributing the fibers about the strand so that the fibers will adhere to the strand.

A further feature of this invention is to pull a continuous strand of material across a fiber collecting surface and through the zone of fiber deposition on the surface by winding the strand around the rotatable member usually employed to pull the body of fibers off the said surface and draft it to the form of a sliver.

The foregoing, as well as other objects, will be made more apparent as this description proceeds, especially when considered in connection with the accompanying drawing, wherein:

2

Figure 1 is a diagrammatic side elevational view partly in section of apparatus constructed in accordance with this invention;

Figure 2 is a sectional view taken substantially on the line 2—2 of Figure 1; and

Figure 3 is a diagrammatic view of the sliver of this invention showing the reinforcing core or strand.

Although this invention concerns itself more particularly with the manufacture of slivers formed of glass, nevertheless, other materials having similar characteristics may be employed. Several examples of materials which may be used in connection with the present invention, are artificial silk commonly known as "nylon," vinyl acetate, cellulose acetate, resin, sugar, and vinylidene chloride resin.

With the above in view reference is now made to the drawing wherein it will be noted that the reference character 10 indicates a container or melter adapted to contain a supply 11 of molten thermoplastic material such as glass. A bushing 12 is suitably supported at the bottom of the container in communication with the supply 11 of molten glass and comprises a plurality of nipples or relatively small orifices 13.

The orifices 13 are designed to enable a glass stream to be drawn through each orifice by a blower 14 supported below the bushing 12 and having the further function of forming attenuated fibers from the glass streams. In detail, the blower 14 comprises complementary sections 15 and 16 respectively positioned at opposite sides of the glass streams issuing from the bushing 12.

The section 16 is provided with a chamber 17 communicating with a source of fluid under pressure, such as a steam or air, by means of a conduit 18 and also communicating at one end with the adjacent end of a chamber 19 formed in the section 15. It will also be noted from Figure 1 that the sections of the blower 14 are respectively formed with discharge orifices arranged to discharge fluid under pressure in a downward direction toward opposite sides of the glass streams. The pressure of the fluid is sufficient to apply the pulling force on the glass streams required to draw the same from their respective orifices and form attenuated glass fibers.

The glass fibers 20 attenuated by the blower 14 are collected in a web on the periphery of a drum 21 suitably supported for rotation beneath the blower 14 in spaced relation to the latter. In accordance with conventional practice the periphery of the drum is perforated and sufficient suction is created in the drum by means not shown

herein to collect the fibers on the periphery of the drum.

The web of fibers collected or disposed on the periphery of the drum is pulled off of the drum by a member 22 supported for rotation at the front side of the drum 21 in spaced relation to the latter. As the web of fibers is pulled off of the drum it is drafted to the form of a sliver 23 and the latter is wound around the rotatable member 22. The fibers produced by the process just described are usually known as staple glass fibers. They are substantially continuous in length when they are formed but are broken up to some extent as they are deposited on the surface of the drum and to greater extent when they are pulled from the surface and drafted into a sliver. The resulting sliver contains, predominantly, fibers of great length but of lengths many times less than the total length of the sliver, with the fibers interlaced and tangled to an extent providing a high degree of integrity in the sliver both in the direction of its length and in transverse directions.

The present invention provides a sliver of this type reinforced with a strand of glass or other fibers. The strand is incorporated in the sliver in such a way that the original fluffy nature of the sliver is not altered as it would be if the strand and the sliver were intertwined or if the sliver was folded about the strand. Retention of the original fluffiness is especially desirable where the sliver is to be served onto a wire to form a layer of fibrous insulation.

To obtain maximum strength in the reinforced sliver it has been found preferable to employ as the reinforcing core a strand or yarn of continuous glass filaments. Glass filaments of the continuous type are made by continuously attenuating streams of molten glass, gathering the fibers thus formed into groups or strands and winding the strands upon a drum or spool. The finished strands contain a large number of filaments that are substantially continuous in length throughout the length of the strand.

The way in which the sliver 23 is reinforced with a strand of material, preferably glass, and either in the form of a strand of glass filaments or in the form of a yarn, will now be described in detail. The reference character 24 in Figure 1 indicates a continuous strand packaged on a spool 25 supported at the rear side of the fiber collecting drum 21. In the present instance, the strand is unwound from the spool 25 by the rotatable member 22 previously described as operable to pull the fibers off the periphery of the collecting drum 21. In the present instance, the strand is passed upwardly through an eye or guide 26 suitably supported above the package 24 and is extended downwardly around a pad 27 to the rotatable member 22. The locations of the pad 27 and the rotatable member 22 with respect to the collecting drum 21 is such as to enable the strand to pass over the collecting drum 21 in contact with the periphery of the latter at the zone of the fiber deposition on the periphery of the drum. The above arrangement is such that the fibers are distributed about the strand as the latter is drawn across the drum 21 by the rotatable member 22 and the strand is felted with the fibers. In accordance with this invention the fibers are secured to the strand by coating the strand with a suitable adhesive prior to moving the strand across the drum 21. In detail, the strand is coated with an adhesive material by the pad 27 and this material is supplied to the pad by a suitable reservoir 28. The adhesive material employed may

be wax, resin, or any similar adhesive capable of securing the fibers to the continuous strand as the latter is drawn through the fiber deposition zone on the drum by the rotatable member 22.

As a result of the above, a sliver of the type shown in Figure 3 of the drawing is produced having a core in the form of a strand such, for example, as a length of glass yarn and having long or theoretically continuous glass fibers interlaced about the core so that the latter acts to effectively reinforce the sliver. It will also be understood from the foregoing that the glass fibers are distributed about the strand by advancing the latter through the zone of fiber deposition on the drum or other fiber collecting surface and, consequently, the relatively long fibers also extend in the general direction of length of the strand but are intertwined to an extent providing integrity in the body of fibers about the core. This arrangement of the fibers around the strand provides a sliver having very high tensile strength and one which will not break during subsequent weaving or knitting operations. Also, by depositing the fibers in tangled relation about the reinforcing strand, the fibers become interlaced about the strand to such an extent that the strand is separated from the body of fibers only with great difficulty, demonstrating the degree of integrity of the product of the present invention.

For some applications of the reinforced sliver it has been found advantageous to employ as a reinforcing core a strand made up of one or more filaments of a thermoplastic resinous material such as Vinylite, polystyrene, "Seran," and similar resins. This is particularly valuable where the sliver is to be served onto a wire to form a layer of insulating material thereover. The sliver is heat treated after it is served on the wire to soften the thermoplastic material of the reinforcing core to an extent causing it to flow and thoroughly impregnate the fibrous insulating layer to provide the needed dielectric resistance.

The thermoplastic core may also be employed where the sliver is to be used for other purposes and wherever it is desired to reinforce the sliver until it has been twisted, woven, knitted, or processed in some other manner, but where the reinforcing is not required after processing but is advantageously replaced by impregnation of the sliver.

Various modifications of the present invention may be made within the spirit of the invention and within the scope of the appended claims.

We claim:

1. Apparatus for forming a reinforced sliver comprising a drum supported for rotation in a position to collect a web of intertwined fibers as it is formed, a package comprising a strand of continuous glass fibers supported at one side of the drum, a rotatable member supported at the opposite side of the drum for pulling the deposited fibers off the periphery of the drum in the direction of rotation of the drum to form a sliver and for also unwinding the package by pulling the strand across the periphery of the drum through the zone of fiber deposition on the drum whereby said fibers are drawn substantially parallel with said strand, means supported adjacent the package in a position to engage the strand as it is unwound from the package and operable to apply an adhesive on the strand to cause the fibers to adhere to the strand as the latter is pulled across the periphery of the drum, and means for applying radially inward forces against said fibers around said strand.

2. The method which comprises continuously forming on the periphery of a rotatable member a glass fiber web in which the fibers are haphazardly arranged and interlaced with each other, advancing a continuous strand of glass fibers across the periphery of said member through the fiber deposition zone on the member and in the direction of its rotation, applying an adhesive to the strand prior to engaging the web to cause the fibers to adhere thereto, and pulling said web and strand together from the periphery of the rotatable member in the general direction of movement of the periphery and at a rate sufficiently higher than the rate of movement of the periphery to draw the fibers of the mat into substantial parallelism with the strand.

3. The method which comprises winding a continuous strand, causing the strand to pass across the periphery of a rotatable member in the direction of its rotation during the winding operation, simultaneously forming and depositing a glass fiber web in which the fibers are haphazardly arranged and interlaced with each other on the periphery of the rotatable member about the strand, and pulling said web and strand together from the periphery of the rotatable member at a rate sufficiently higher than the rate of movement of the periphery to draw the fibers of the mat into substantial parallelism with the strand.

4. The method of forming a reinforced strand or sliver which comprises projecting fine glass filaments onto a moving supporting surface and causing them to accumulate in matted form on said surface with the filaments extending promiscuously and haphazardly but in directions mainly substantially parallel with said surface, continuously passing a preformed strand along said surface in the direction of movement thereof, and continuously drawing the mat of filaments and the strand from said surface as the mat is formed at a rate greater than the rate of movement of said surface, and simultaneously transforming the mat into the form of a reinforced strand or sliver in which the filaments are arranged mainly in substantial parallelism about said strand.

5. The method of forming a reinforced strand or sliver which comprises projecting fine glass

filaments onto a moving supporting surface and causing them to accumulate in matted form on said surface with the filaments extending promiscuously and haphazardly but in directions mainly substantially parallel with said surface, continuously passing a preformed strand along said surface in the direction of movement thereof, and continuously drawing the mat of filaments and the strand from said surface as the mat is formed, at a rate greater than the rate of movement of said surface, whereby the mat of filaments is attenuated as it is drawn together with the strand from said surface, and concentrating the mat of filaments to compact sliver form about the strand as it advances beyond said surface.

6. Apparatus for forming a reinforced sliver comprising a drum supported for rotation in a position to collect a web of intertwined fibers as it is formed, means for supporting a package comprising a strand of continuous glass fibers at one side of the drum, a rotatable member supported at the opposite side of the drum for pulling the deposited fibers off the periphery of the drum in the direction of rotation of the drum to form a sliver and for also unwinding the said package by pulling the strand across the periphery of the drum through the zone of fiber deposition on the drum, whereby said fibers are drawn substantially parallel with said strand, and means for applying 30 radially inward forces against said fibers around said strand.

7. The method which comprises winding a continuous strand of thermoplastic resinous material, causing the strand to pass across the periphery of a rotatable member in the direction of its rotation during the winding operation, simultaneously forming and depositing a glass fiber web in which the fibers are haphazardly arranged and interlaced with each other on the periphery of the rotatable member about the strand, and pulling said web and strand together from the periphery of the rotatable member at a rate sufficiently higher than the rate of movement of the periphery to draw the fibers of the mat into substantial parallelism with the strand.

JAMES R. McMILLIN.  
STANLEY H. LAKE.